

Oct. 12, 1926.

1,602,795

W. E. GREENAWALT

## METALLURGICAL PROCESSES

Filed Jan. 31, 1925



Fic 1



FIG 2

INVENTOR  
William E. Greenawalt?

Patented Oct. 12, 1926.

1,602,795

# UNITED STATES PATENT OFFICE.

WILLIAM E. GREENAWALT, OF DENVER, COLORADO.

## METALLURGICAL PROCESS.

Application filed January 31, 1925. Serial No. 6,112.

The invention is more specifically directed to the extraction of copper from its ores and the precipitation of the dissolved copper from the resulting solutions, either in whole 5 or in part, with hydrogen sulphide. It may be considered as an improvement, or more or less specific application, of the more general process patented by me March 6, 1917, No. 1,218,177, although it is not intended to limit 10 its use to any particular application.

The process has as its object the production of metallic copper from its ores without resorting to regular smelting and refining methods, which, in most mining districts, are 15 too expensive for general adoption, especially on a small scale.

The present process is an attempt to combine hydrometallurgy with pyrometallurgy, preferably using the electric current for 20 both, in such a way as to give a distinct advantage over either method taken separately, on certain classes of copper ore.

The following considerations are the principal factors governing the process, and 25 when these are understood, the process can easily be comprehended.

Most mines, or mining districts, produce 30 large amounts of low grade copper ore, usually in the form of sulphide, or as the sulphide and oxide (including carbonate) mixed. In either case the general method of procedure is to separate the sulphide mineral from the gangue to form a concentrate. This concentrate is usually of relatively low 35 grade, as compared with the theoretical percentage of copper in the mineralogical combination of the copper minerals. Considerable gangue is associated with the copper in the concentrate, and usually a large amount 40 of iron, either as pyrites, or combined mineralogically with the copper, as in chalcopyrite and bornite. Quite generally chalcocite, having the mineralogical formula of  $Cu_2S$ , will form a constituent of the various copper 45 ores, and to some extent also covellite, which has the mineralogical formula of  $CuS$ .

In the concentration treatment of copper ores, the concentrate is usually so contaminated with iron, silica, alumina, etc., that 50 vigorous fluxing is required for good smelting conditions, and this makes a smelting process expensive to install and expensive to operate. Where power is cheap and fuel is costly electric smelting would appear to 55 present some advantages, but the complications arising from the fluxing of large quan-

tities of material and the large amount of electricity required, has led to failure or disappointment wherever it has been tried.

In the concentration treatment of mine 60 ore, either by gravity or flotation, a certain amount of very high grade concentrate may be separated from the large amount of the ordinary sulphide concentrate, but the relatively small amount of very high grade concentrate 65 will contain a relatively large portion of the total copper. Usually this relatively small portion of high grade concentrate will be in the form of chalcocite, with probably relatively small amounts of chalcopyrite and bornite, which will contaminate the high grade concentrate with a small amount of iron, but not enough to seriously affect the present process.

The copper, in what is known as the porphyry, or disseminated, deposits, is largely in the form of chalcocite,  $Cu_2S$ , and containing, theoretically, 79.8% copper and 20.2% sulphur.

The conditions of concentration can best 75 be illustrated by taking a specific case in the treatment of 100 tons of ore assaying 1.5%, or 30 lbs. of copper per ton, or containing a total of 3000 lbs. of copper. If 80 the ratio of concentration is 10 into 1, we would have, as the result of the concentration treatment: 90 tons tailing, 0.25% copper (5 lbs.), 450 lbs. total; 10 tons concentrate, 12.75% copper (255 lbs.), 2550 lbs. 85 total.

The ten tons of concentrate may then be separated into: 1.5 tons high grade concentrate, 50% copper (1000 lbs.), 1500 lbs. total; 8.5 tons low grade concentrate, 6.2% copper (124 lbs.), 1050 lbs. total.

Or, preferably, into the following: 1.0 ton high grade concentrate, 60% copper (1200 lbs.), 1200 lbs. total; 9.0 tons low grade concentrate, 7.5% copper (150 lbs.), 100 1350 lbs. total.

There should be no difficulty in making a relatively small amount of high grade concentrate, if much of the copper in the ore is in the form of chalcocite. For a 50% copper 105 concentrate, there would be a margin of 29.8% of the theoretical; and for a 60% copper concentrate, there would be a margin of 19.0% of the theoretical. The latter is preferred and will be assumed for illustration, altho it will be understood that the process is not particularly limited to the percentage of copper in the high grade con-

centrate, but that the higher the grade of the high grade copper concentrate, the better the process can be operated. A ton of 60% copper concentrate would contain, 5 approximately, copper, 1200 lbs.; sulphur, 400 lbs.; impurities, 400 lbs.

The impurities may be assumed to be mostly iron, with its combined sulphur, silica and alumina, and combined oxygen.

10 If there is gold or silver in the ore, the high grade concentrate will contain the precious metals in about the same proportion as it contains the copper from the original ore. That is to say, of the total precious 15 metal content in the concentrate, 47.5% will be in the one ton of 60% copper concentrate, and 52.5% will be in the 9.0 tons of 7.5% copper concentrate.

Having made the separation of the mineral from the gangue and divided the mineral into a relatively small amount of high grade concentrate and a relatively large amount of low grade concentrate, the 20 method of procedure is as follows, reference being made to the accompanying drawings, in which Fig. 1 is a diagrammatic flow sheet in plan of the process, and Fig. 2 is a diagrammatic flow sheet in section of that portion of the process which relates to 25 the treatment of the high-grade concentrate and the production of the precipitant for the copper from its solutions, and the application of the precipitant to the copper solutions.

30 The low grade copper concentrate is roasted so as to convert as much as possible of the copper into sulphate, which is soluble in water, and which makes possible a high extraction of the copper from the roasted material by water and by acid leaching, and supplies the necessary acid for the process. The roasted low grade concentrate is then leached with a dilute acid solution, and the resulting copper solution, containing salts 35 of iron, is then electrolyzed to deposit the copper, while at the same time acid and ferric salts are regenerated. In order to avoid the harmful effects of the ferric iron in the electrolyte the sulphur dioxide from the 40 roasting furnace is applied to the electrolyzed solution by which means the ferric iron, produced by the electrolytic deposition of the copper, is maintained within fairly harmless limits. The copper solution 45 from the leaching tank flows into the  $\text{SO}_2$  reducer No. 1, and from the reducer into the electrolytic copper tanks No. 1. If desired, the solution may be treated with  $\text{CuS}$  precipitate obtained from waste and foul 50 solutions, in the  $\text{CuS}$  reducer, as will be referred to later.

55 The solution is flowed through the electrolytic copper tanks at a rate which experience has shown to be the most satisfactory in reference to the formation of ferric iron

in the electrolyte in the deposition of the copper from solution containing salts of iron. Usually the amount of ferric iron in the solution issuing from the electrolytic copper tanks should not exceed about 0.25%, altho 70 there is no definite rule in this respect. The solution is circulated in a sort of closed circuit between the  $\text{SO}_2$  reducer and the electrolytic copper tanks No. 1, until the desired amount of copper is removed from the 75 solution, which, in the case of a 3.50% copper solution, would be about 1.5%, leaving about 2.0% in the solution, assuming two electrolytic and reduction circuits as shown in the drawing.

80 A regulated stream of solution—the regular advance flow through the leaching and electrolytic circuit—is passed on to the second electrolytic unit, comprising the  $\text{SO}_2$  reducer No. 2 and the electrolytic copper tanks 85 No. 2, where more copper is deposited and more acid and ferric iron regenerated, and the cycle of electrolysis and reduction is continued in the second electrolytic unit until the desired amount of copper has been removed, which, for the assumed solution, would be about 1.0% removed, and about 90 1.0% remaining in the solution. A portion of the depleted copper solution—the advance flow—regenerated in acid, is then returned 95 to the ore to pass through another complete cycle of leaching and copper deposition and acid regeneration, and this is continued indefinitely. When one lot of ore or concentrate is treated, the solution is switched to 100 a new charge. In this way the copper is extracted from the low grade concentrate and converted into the electrolytic metal.

105 Manifestly, if this cycle of solution and precipitation is continued, the solution will become charged with iron and other impurities in a short time so as to make its use undesirable, either as a solvent or as an electrolyte. A certain amount of foul solution is therefore diverted from the leaching and electrolytic circuit and wasted, while an equivalent amount of wash water is added to the solution to make up the loss in the regular operation of the process.

110 The copper in the foul solution, diverted from the leaching and electrolytic circuit, is precipitated before the solution is wasted, preferably with hydrogen sulphide.

115 The generation of hydrogen sulphide for copper precipitation purposes has always 120 presented something of a problem in its commercial application. Hydrogen sulphide for commercial use is ordinarily generated from ferrous sulphide, or iron matte, and acid, but this method is rather expensive 125 in copper mining districts. It involves the purchase or special manufacture of acid for this purpose, and that should be avoided if possible. The general process, as described, is usually self sustaining in acid; that is to 130

say, there is as much acid generated in the steps of roasting, leaching, reduction, and electrolysis, as is required to dissolve the copper from the ore, without resorting to special acid manufacture or purchase. In such a case it would be particularly desirable if the precipitation of the copper from the lean and foul solutions could be accomplished with a precipitant, such as hydrogen sulphide, produced from the ore itself, as a step in the recovery of the copper.

According to the present process this is accomplished by separating a relatively small amount of high grade concentrate from a relatively large amount of low grade concentrate, and then using the high grade concentrate as a source of hydrogen sulphide to precipitate the copper from solutions obtained in leaching the low grade concentrate or low grade ore, especially from the lean and waste foul solutions.

The low grade concentrate is preferably treated by roasting, leaching, reduction, and electrolysis, as described. The relatively small amount of high grade concentrate is heated in an electric furnace in a neutral or in a reducing atmosphere to dissociate the copper sulphide into its constituent elements, sulphur and copper. A high temperature is necessary for the complete dissociation of the copper and sulphur of the sulphide concentrate. Cuprous sulphide,  $Cu_2S$ , when heated to redness in the presence of steam is but slightly decomposed, but at the white heat easily obtainable in an electric furnace in a non-oxidizing atmosphere, the cuprous sulphide is dissociated, in the presence of steam, with the result, that large quantities of hydrogen and hydrogen sulphide together with sublimed sulphur are evolved, and the copper is completely reduced to the metallic state. The reduction of the cupric sulphide,  $CuS$ , to the cuprous sulphide,  $Cu_2S$ , takes place at a considerably lower temperature than that required for the dissociation of the cuprous sulphide, but as the object is to obtain hydrogen sulphide and metallic copper from the high grade concentrate, a high temperature is required to complete the reduction.

The cuprous sulphide, once heated, requires only a relatively small amount of additional heat to maintain it at the dissociation temperature. The rapidity of dissociation of the cuprous sulphide is governed by the temperature, and the temperature is regulated by the electric current.

Hydrogen sulphide begins to dissociate at about 400 deg. C., and increases with the rise in temperature. Careful regulation of the escaping gases is important, and the temperature of the gases should not greatly exceed 500 deg. C. to prevent the dissociation of the hydrogen sulphide.

While the regulation of the temperature

of the cuprous sulphide in the electric furnace is quite easy, the regulation of the temperature of the gases in the furnace is quite difficult, if not impossible, to get the maximum amount of hydrogen sulphide with a minimum amount of free hydrogen and free sulphur.

To meet this condition, the gases escaping from the electric furnace are passed through the  $H_2S$  rectifier, where the conditions for the maximum production of hydrogen sulphide can be controlled and regulated. The temperature may be maintained to get the maximum formation of hydrogen sulphide from the uncombined hydrogen and sulphur vapor, with the minimum amount of disintegration of the hydrogen sulphide. In addition to the close regulation of temperature, the rectifier may and usually will contain material which promotes the formation of hydrogen sulphide, such as pumice or glass, either of which appears to act as a catalyst. The rectifier may consist of a tube or chamber, containing a catalyst, such as pumice, which may be heated indirectly through the walls of the chamber, or directly by an electric current, to the desired temperature, or say, from 400 to 500 deg. C. The mixture of hydrogen sulphide, hydrogen, and sulphur vapor from the electric furnace is passed through the rectifier to combine the uncombined hydrogen with the uncombined sulphur vapor to form an equivalent of hydrogen sulphide. The gas is then used to precipitate the copper or other metals from solutions, especially from waste foul copper solutions and lean wash waters.

In the production of hydrogen sulphide, either in the electric furnace or in the  $H_2S$  rectifier, a hydrocarbon, preferably in the form of oil, may be used with or without steam and forms a convenient way of supplying hydrogen or a hydrogen containing fluid and maintaining the reducing atmosphere desired for good operating conditions. Excellent results can be obtained by introducing hydrogen or a hydrogen containing gas into the electric furnace or into the rectifier, but such gases are expensive to produce in copper mining districts, and oil will usually be preferred. The source of hydrogen which is best available for any particular condition would naturally be used.

The hydrogen sulphide is applied to the copper solutions, preferably to the diverted foul solutions and lean wash waters, in the  $H_2S$  precipitator, where the copper and some of the other metals are precipitated from the solutions, with the simultaneous regeneration of acid. The solution, with the copper sulphide in suspension, flows into the  $CuS$  separator, where the  $CuS$  is separated from the barren solution. The  $CuS$  is preferably applied to the electrolyte of the leaching and electrolytic circuit, where it may be

used to reduce the ferric iron produced by the electrolytic deposition of the copper to the ferrous condition, while at the same time the copper of the precipitate is converted 5 into the electrolytic metal, as described more fully in my Patents No. 1,340,826, May 18, 1920, and No. 1,357,495, Nov. 2, 1920.

The barren foul acid solution and wash waters may be wasted, but if there is oxidized ore available for leaching, these foul and dilute acid solutions are advantageously used in leaching the copper from the oxidized ore. This oxidized ore will frequently consist of the tailings from the preliminary 10 concentration treatment for obtaining sulphide concentrates.

When the copper sulphide in the electric furnace has been reduced to metallic copper, it is drawn from the furnace and given 20 any further desired treatment. It is preferred however to cast this impure copper into anodes and then place the copper anodes in the electrolytic copper tanks, using the leach copper solution as the electrolyte, and 25 thus the impure copper from the electric furnace may be converted into the pure electrolytic metal at very little additional expense. The precious metals in the copper from the electric furnace are recovered from the insoluble residue in the electrolytic copper 30 tanks. The electrolytic copper tanks may therefore be used to deposit copper from the leach solutions, to refine the impure copper from the electric furnace, or both at the 35 same time in different tanks. This can be done quite conveniently if suitable provision is made to take care of the difference in the E. M. F. required for the deposition of copper from insoluble anodes and from soluble 40 anodes. The E. M. F. required to deposit the copper from leach solution, with lead anodes for example, will usually vary from 1.5 to 1.9 volts, while with soluble or copper 45 anodes for example, the E. M. F. will usually vary from 0.2 to 0.3 volt, under the conditions assumed. The amount of copper deposited, per ampere, will be about the same in either case.

It is desirable to have a high grade copper concentrate for treatment in the electric furnace for the reason that a large amount of impurity would interfere with getting good reacting conditions between the sulphur vapor and the hydrogen containing 50 fluid to form hydrogen sulphide. If the copper concentrate contained a large amount of impurity, a procedure akin to that of smelting would have to be resorted to, and this would involve vigorous fluxing and the 55 separation and removal of the resulting slag. Even with a high grade concentrate some slag will form and will have to be removed. It is largely to avoid this complication in 60 connection with the production of hydrogen sulphide that the amount of impurity is

maintained as low as possible. Evidently also, a high grade concentrate will require less attendance, and if the concentrate is of very high grade, as preferred, the operation may proceed with a small amount of care or 70 supervision. Another reason for preferring a high grade concentrate is that a small electric furnace, and hence a simple equipment, is capable of a relatively large output of copper. An electric furnace having a 75 charge dimension of only 2 x 2 x 2 feet, or 3 x 3 x 1 foot, would take a charge of a ton of concentrate, assuming the weight of the concentrate to be about 250 lbs. per cubic foot. Each charge would produce about 1200 lbs. 80 of copper, under the assumed conditions of a 60% copper concentrate.

In case the ore is such that a high grade concentrate is not obtainable direct from the ore either by gravity or flotation, as 85 would be the case if the ore is largely pyritic and the copper in the form of chalcopyrite or bornite, with a consequent large amount of gangue, it is preferred to smelt this medium grade ore or concentrate to slag off 90 the iron, silica, and other impurities, and then to introduce the resulting high grade copper sulphide in molten form into the electric furnace for the production of hydrogen sulphide and metallic copper. In 95 this also, only a very small smelting equipment would be necessary for a relatively large output of copper from a concentrate containing say, from 40% to 50% copper. Under such conditions there would not be 100 any difficulty in getting a relatively pure copper sulphide for the electric furnace. Small smelting furnaces are usually somewhat impractical on ordinary low grade copper ores, but small units are quite practical when smelting a well fluxed high or 105 medium grade concentrate.

Theoretically, the sulphur combined with the copper as  $Cu_2S$ , in the high grade concentrate will combine with the copper of the precipitate as  $CuS$ ; or, one ton of copper will be produced in the electric furnace in the precipitation of half a ton of copper from the leach solutions. From this it will 110 be seen that a suitable working relation can easily be established between the high grade and the low grade concentrate, and between the relative amounts of copper to be produced by leaching and by electric smelting.

It will also be noticed that by this method of precipitating copper from leach solutions, the precipitant,  $H_2S$ , is produced at a very small, or practically no extra expense, for it is believed that the electric smelting of 115 the relatively high grade concentrate, where possible, offers certain advantages over treating the same material by any other method, either hydro or pyro metallurgically. Such an electric smelting process 120

would not of itself offer any advantage in the ordinary treatment of copper ore or concentrate for the reason that the treatment of the lower grade material would still have 5 to be dealt with, and the lower grade material, in any case, offers the most difficult problem, either by itself, or in relation to other steps.

In case sulphur in suitable form for the 10 electric furnace is scarce, sulphur vapor, or even sulphur dioxide, may be introduced into the electric furnace or into the  $H_2S$  rectifier. Coke may be placed on top of the charge in the electric furnace, or placed in 15 the rectifier, if desired, to give the desired reducing atmosphere.

Similarly, if sulphur in any form is scarce, the  $CuS$  of the precipitate may be used in the electric furnace, and the sulphur used 20 cyclically in precipitation, while the copper of the precipitate would be converted into the metallic state. It is preferred, however, to use the  $CuS$  precipitate for reducing ferric iron in the electrolyte since this offers 25 a more satisfactory way to convert the copper of the precipitate into the electrolytic metal. Again, drying and melting of a voluminous precipitate, such as  $CuS$ , is bothersome, while by using it as a reducing 30 agent in the electrolyte, the handling of the precipitate is very simple and can be done at very small extra cost.

The process has been described more particularly in reference to the treatment of 35 copper ores for which it is primarily intended and to which it is eminently adapted. It is evident, however, that it is applicable to other ores.

I claim:

40 1. A process of treating copper ores comprising, concentrating the ore into a relatively small amount of high grade sulphide concentrate and a relatively large amount of low grade concentrate, roasting the low grade concentrate, leaching the roasted low grade concentrate with a suitable solvent for the copper, heating the high grade sulphide concentrate to dissociate the combined copper and sulphur, applying a hydrogen containing fluid to the resulting sulphur vapor to form hydrogen sulphide, and precipitating copper from the leach solution with the hydrogen sulphide.

45 2. A process of treating copper ores comprising, concentrating the ore into a low grade concentrate and into a high grade sulphide concentrate, leaching the low grade concentrate with a suitable solvent for the copper, heating the high grade sulphide concentrate to dissociate the combined copper and sulphur, passing the resulting sulphur vapor through a rectifier or chamber in the presence of a hydrogen containing fluid maintained at a temperature to combine the hydrogen with the sulphur vapor to form

hydrogen sulphide, and precipitating copper from the leach solution from the low grade concentrate with the hydrogen sulphide so obtained from the high grade concentrate.

70

3. A process of treating copper ores comprising, concentrating the ore to remove a portion of the copper as a relatively high grade sulphide concentrate, leaching the low grade material from which the high grade 75 concentrate was separated with a suitable solvent for the copper, heating the high grade concentrate to dissociate the combined copper and sulphur, applying a hydrogen containing fluid to the resulting sulphur vapor to form hydrogen sulphide, and then precipitating copper from the copper solutions obtained from leaching the low grade material with the hydrogen sulphide so obtained from the high grade concentrate.

80

4. A process of treating copper ores comprising, concentrating the ore to remove a portion of the copper as a relatively high grade concentrate, leaching low grade copper bearing material with an acid solution to 90 extract the copper, electrolyzing the resulting copper solution to deposit the copper and regenerate acid, returning the regenerated acid solution to the ore and repeating the cycle of leaching and electrolysis until the 95 solution becomes fouled with impurities, heating the high grade sulphide concentrate to dissociate the combined copper and sulphur, applying a hydrogen containing fluid to the resulting sulphur vapor to form hydrogen sulphide, and then precipitating the copper from the foul leach solution from the low grade copper bearing material with said hydrogen sulphide.

100

5. A process of treating copper ores comprising, concentrating the ore to remove a portion of the copper as a relatively high grade sulphide concentrate, leaching low grade copper bearing material with an acid solution to extract the copper and regenerate 105 acid and then returning the acid solution to the ore or low grade copper bearing material, heating the high grade sulphide concentrate to dissociate the combined copper and sulphur, applying a hydrogen containing fluid to the resulting sulphur vapor to 110 form hydrogen sulphide, applying the hydrogen sulphide so produced to the foul electrolyzed solution resulting from leaching the low grade material, casting the resulting copper from the high grade concentrate into suitable anodes, and then refining said anodes in the copper electrolyte in the leaching and electrolytic circuit.

115

6. A process of treating copper ores comprising, concentrating the ore into a relatively small amount of high grade sulphide concentrate and a relatively large amount of low grade concentrate, roasting the low grade concentrate, leaching the roasted low

125

130

- grade concentrate with an acid solution to extract the copper, electrolyzing the resulting copper solution to deposit the copper and regenerate acid, returning the regenerated acid solution to the roasted low grade concentrate and repeating the cycle until the copper in the low grade concentrate is sufficiently extracted, heating the high grade concentrate to dissociate the combined copper and sulphur, casting the resulting impure copper from the high grade concentrate into anodes, and refining said anodes in the electrolyte or solution obtained from leaching the low grade concentrate.
- 15 7. A process of treating copper ores comprising, concentrating the ore to remove a portion of the copper as a sulphide concentrate, leaching low grade copper bearing material with an acid solution to extract the
- 20 copper, smelting the sulphide concentrate to remove impurities and to obtain a high grade copper sulphide, heating the copper sulphide in an electric furnace in a reducing atmosphere to dissociate the combined copper and sulphur, applying a hydrogen containing fluid to the resulting sulphur vapor to form hydrogen sulphide, and then precipitating copper from the leach copper solution with said hydrogen sulphide.
- 25 8. A metallurgical process comprising, concentrating ores of metals to remove a relatively high grade sulphide concentrate, leaching the resulting low grade material with a suitable solvent to extract the metals, heating the high grade concentrate in an electric furnace in a reducing atmosphere to drive off the sulphur, passing the resulting sulphur vapor together with a hydrogen containing gas through a rectifier or chamber maintained at the desired temperature to combine the sulphur and the hydrogen to form hydrogen sulphide, and then precipitating metals from the leach solution with said hydrogen sulphide.
- 30 9. A metallurgical process comprising, concentrating copper ore to remove a relatively high grade sulphide concentrate, leaching the resulting low grade material with a suitable solvent to extract the copper, heating the sulphide concentrate in an electric furnace to dissociate the combined copper and sulphur, applying a hydrogen containing fluid to the resulting sulphur vapor in the presence of a catalytic agent to combine the sulphur and hydrogen to form hydrogen sulphide, and then precipitating copper from the leach solutions with said hydrogen sulphide.
- 35 10. A metallurgical process comprising, concentrating ores of metals to remove a high grade sulphide concentrate, leaching relatively low grade ores of the metals with a suitable solvent for the metals, heating the high grade sulphide concentrate in an electric furnace to dissociate the sulphur, and

then as a separate step combining the dissociated sulphur with hydrogen in the presence of a substance capable of promoting the reaction between the sulphur vapor and a hydrogen containing fluid to produce hydrogen sulphide, and then precipitating metals from the leach solution with said hydrogen sulphide.

11. In the production of hydrogen sulphide for precipitating metals from leach solutions the steps comprising, heating a sulphide concentrate in a reducing atmosphere to dissociate the sulphur, then as a separate step from said heating and dissociation combining the resulting sulphur vapor with hydrogen in the presence of a catalytic agent heated to the reacting temperature between sulphur and hydrogen to form hydrogen sulphide.

12. A metallurgical process comprising, leaching low grade ores of metals with a suitable solvent for the metals, heating a sulphide concentrate in a reducing atmosphere in an electric furnace to dissociate the copper and the sulphur, then as a separate step from said heating and dissociation combining the resulting sulphur vapor with hydrogen to form hydrogen sulphide in the presence of a substance capable of promoting the reaction while subjecting said substance to the action of an electric current, and precipitating metals from the leach solution with the hydrogen sulphide so formed.

13. A metallurgical process comprising, leaching low grade ores of metals with a suitable solvent for the metals, treating a sulphur containing substance in a reducing atmosphere to form sulphur vapor, then as a separate step from said formation of sulphur vapor combining the sulphur vapor with hydrogen to form hydrogen sulphide by heating the sulphur vapor and hydrogen containing fluid to a reacting temperature in the presence of a catalytic agent capable of promoting the reaction, and then precipitating metals from the leach solutions with the hydrogen sulphide so formed.

14. A process of treating copper ores comprising, concentrating the ore into a relatively small amount of high grade sulphide concentrate and a relatively large amount of low grade concentrate, roasting the low grade concentrate, leaching the roasted low grade concentrate with a dilute acid solution to extract the copper, electrolyzing the resulting copper solution to deposit the copper and regenerate acid, returning the regenerated acid solution to the ore and repeating the cycle of leaching and electrolysis until the copper in the roasted concentrate is sufficiently extracted, heating the high grade sulphide concentrate to dissociate the combined copper and sulphur, combining the resulting sulphur vapor with hydrogen to form hydrogen sulphide, precipitating the

- 5 copper from the foul electrolyzed solutions with hydrogen sulphide, applying the CuS precipitate to the electrolyte, and applying the impure copper from the high grade concentrate to the electrolyte as anodes to convert it into the electrolytic metal.
- 10 15. A process of treating copper ores comprising, concentrating the ore into a relatively small amount of high grade sulphide concentrate, leaching a low grade copper ore with a suitable solvent to extract the copper, heating the high grade sulphide concentrate to dissociate the combined copper and sulphur, passing the resulting sulphur vapor and a hydrogen containing fluid through the interstices of an incandescent mass of material such as pumice, coke, or glass, which is capable of promoting the combining reaction between the sulphur and the hydrogen to form hydrogen sulphide, and then precipitating copper from the leach solution with said hydrogen sulphide.
- 15 20 25 30 35 40 45 50 55 60 65 70 75 80 85 90 95 100 105 110 115 120 125 130
16. A process of treating copper ores comprising, leaching ores of copper with an acid solution to extract the copper, treating a sulphur containing substance by heating it in a reducing atmosphere to convert the sulphur of the substance into sulphur vapor, then passing the sulphur vapor with a hydrogen containing fluid through the interstices of a mass of a catalytic agent composed of pieces and heated to incandescence in a reducing atmosphere to combine the sulphur with the hydrogen to form hydrogen sulphide, and then precipitating copper from the leach solutions with said hydrogen sulphide.
17. A process of treating copper ores comprising, concentrating the ore into a relatively small amount of high grade concentrate and a relatively large amount of low grade material, leaching the low grade material with a suitable solvent for the copper, heating the high grade sulphide concentrate in an electric furnace in a reducing atmosphere to dissociate the copper and sulphur, introducing steam into the electric furnace, passing the resulting mixture of sulphur vapor, steam, hydrogen, and hydrogen sulphide, through the interstices of a mass of incandescent material such as pumice, coke, or glass, to complete the formation of hydrogen sulphide from the uncombined sulphur vapor and hydrogen, then precipitating copper from the leach solutions with said hydrogen sulphide.
18. A process of treating mixed sulphide and oxide ores of copper comprising, separating the pulverized ore by gravity or flotation concentration into a high grade sulphide concentrate, a low grade concentrate, and an oxidized tailing, roasting the low grade concentrate, leaching the roasted low grade concentrate with a dilute acid solution to dissolve the copper, electrolyzing the resulting copper solution to deposit the copper and regenerate acid, returning the regenerated acid solution to the roasted concentrate and repeating the cycle whereby excess acid is produced, leaching the oxidized tailing with the excess acid produced by the electrolysis of the leach solution from the roasted concentrate, heating the high grade sulphide concentrate to dissociate the copper and sulphur, applying a hydrogen containing fluid to the resulting sulphur vapor to form hydrogen sulphide, and then precipitating copper from waste foul solutions and lean wash waters obtained from leaching the roasted concentrate and oxidized tailing with said hydrogen sulphide.
19. A process of treating mixed sulphide and oxide ores of copper comprising, separating the pulverized ore by gravity or flotation concentration into a high grade sulphide concentrate, a low grade concentrate, and an oxidized tailing, roasting the low grade concentrate, leaching the roasted concentrate with a dilute acid solution to dissolve the copper, electrolyzing the resulting solution to deposit the copper and regenerate acid, returning the acid solution to the roasted concentrate and repeating the cycle whereby excess acid is produced, leaching the oxidized tailing with the excess acid produced, heating the high grade sulphide concentrate in an electric furnace to dissociate the copper and sulphur, refining said copper with the leach solution as an electrolyte, combining the liberated sulphur with hydrogen to form hydrogen sulphide, precipitating copper from the foul leach solutions and wash waters with said hydrogen sulphide, and treating the electrolyte with the resulting copper precipitate.
20. A process of treating copper ores comprising, concentrating the ore into a relatively small amount of high grade sulphide concentrate and a relatively large amount of low grade concentrate, roasting the low grade concentrate, leaching the roasted low grade concentrate with an acid solution, electrolyzing the resulting copper solution containing salts of iron to deposit the copper and regenerate acid and ferric iron and returning the electrolyzed solution to the roasted concentrate, applying the sulphur dioxide from roasting the low grade concentrate to the electrolyte as a reducing agent for the ferric iron formed by the electrolysis, heating the high grade sulphide concentrate to dissociate the copper and sulphur, combining the dissociated sulphur with hydrogen to form hydrogen sulphide, and using said hydrogen sulphide as a precipitating agent for copper in the foul and lean leach solutions obtained in treating the low grade concentrate.
21. A metallurgical process comprising, concentrating copper ore to obtain a rel-

- atively high grade copper sulphide concentrate, leaching copper ore with a suitable solvent to extract the copper, heating the sulphide copper concentrate in an electric furnace to dissociate the combined copper and sulphur, combining the resulting sulphur vapor with a gaseous element, and applying the resulting sulphur compound to the leach copper solution.
22. A metallurgical process comprising, concentrating copper ore into a relatively high grade sulphide concentrate and a relatively low grade residue, leaching the relatively low grade residue with an acid solution to extract the copper, electrolyzing the resulting copper solution to deposit the copper and regenerate acid, returning the regenerated acid solution to the low grade residue and repeating the cycle, heating the high grade sulphide copper concentrate in an electric furnace to dissociate the combined copper and sulphur, combining the resulting sulphur vapor with a gaseous element to form a reducing gas, and applying the reducing gas to the copper leach solution as a reducing or a precipitation agent.
23. A process comprising concentrating copper ore into a low grade and a high grade concentrate, roasting the low grade concentrate, leaching the roasted low grade concentrate with an acid solution to extract the copper, electrolyzing the resulting copper solution to deposit the copper and regenerate acid and returning the regenerated acid solution to the roasted low grade concentrate, fusing the unroasted high grade concentrate to eliminate sulphur and slag off impurities, dissolving the copper from the resulting fused copper product in the solution obtained from leaching the roasted low grade
- concentrate, and depositing the dissolved copper as the electrolytic metal.
24. A metallurgical process comprising, concentrating copper ore into a high grade and a low grade concentrate, roasting the low grade concentrate, leaching the roasted low grade concentrate with a dilute acid solution to extract the copper, electrolyzing the resulting copper solution to deposit the copper, fusing the high grade concentrate to still further concentrate it by eliminating sulphur and slagging off impurities, casting the resulting fused concentrated copper product into anodes, and refining said anodes in the solution obtained from leaching the roasted low grade copper concentrate as an electrolyte.
25. A metallurgical process comprising, concentrating copper ore into a high grade and a low grade concentrate, roasting the low grade concentrate, leaching the roasted low grade concentrate with a dilute acid solution to extract the copper, electrolyzing the resulting copper solution to deposit the copper, fusing the high grade copper concentrate in an electric furnace in a non-oxidizing atmosphere to still further concentrate it by eliminating sulphur and slagging off impurities, casting the resulting fused concentrated copper product into anodes, refining said anodes in the copper solution obtained from leaching the roasted low grade concentrate as an electrolyte, combining the sulphur vapor from the electric furnace with hydrogen to form hydrogen sulphide, and applying said hydrogen sulphide to lean and foul leach copper solutions to precipitate the copper therefrom.

WILLIAM E. GREENAWALT.